# EUROPEAN PATENT SPECIFICATION

(11) **EP 1 967 622 B1**
(45) Date of publication and mention of the grant of the patent: **25.08.2010**
(21) Application number: 08102250.1
(22) Date of filing: 04.03.2008
(51) Int. Cl.: D03D 15/00, D03D 15/06, D02G 3/02, D02G 3/04, D02G 3/22, D02G 3/28, D02G 3/38, D02G 3/40

(54) **Process for the production of a textile in extra-fine animal fibres which are not industrially weavable, by the use of continuous water-soluble synthetic filaments**
Verfahren zur Herstellung eines Gewebes aus extrafeinen Tierfasern, die nicht industriell webbar sind, durch Verwendung kontinuierlicher und synthetischer wasserlöslicher Garne
Procédé pour la production d'un textile avec des fibres d'animal extra-fines qui ne peuvent pas être tissées à l'échelle industrielle, à l'aide de filaments synthétiques continus solubles dans l'eau

(30) Priority: 09.03.2007 IT MI20070467
(43) Date of publication of application: 10.09.2008
(73) Proprietor: Geraldini, Jacopo, 20122 Milano (IT)
(72) Inventor: Geraldini, Jacopo, 20122 Milano (IT)
(74) Representative: Mittler, Enrico

(56) References cited:
- EP-A- 1 061 162
- EP-A- 1 245 706
- EP-A- 1 411 160
- EP-A2- 1 953 280
- GB-A- 1 068 662
- JP-A- 55 098 936
- US-A- 2 592 153

## Description

The present invention concerns a process for the production of a textile in extra-fine animal fibres which are not industrially weavable.

In the field of extra-fine animal fibres it is well-known that it is possible industrially to manufacture yarns of very high fineness, for example worsted yarns with a fineness of between 50 and 200 dtex. It is however equally well-known that such yarns have a kinetic strength so low as not to be able to undergo an industrial weaving operation at single ply, which requires a breaking strength of not less than 80-100 grams.

To solve this problem, it has already been proposed by the same Applicant, according to European Patent no. 1 061 162, to double a yarn of pure extra-fine cashmere fibres and a yarn of water-soluble synthetic fibres (or, better, soluble in a slightly acidic aqueous solution at high temperature), to then weave the doubled yarns thus obtained, and finally to dissolve the water-soluble yarns in order to obtain a final textile of pure extra-fine cashmere.

According to this process, starting from yarns of pure cashmere fibres with a Z twist, the doubling is carried out with an opposite twist to that of the individual yarn, i.e. with an S twist, so as to avoid twists which the yarns of extra-fine cashmere fibres cannot tolerate, and thus obtain a final textile that is extremely soft and pleasant to the touch.

Alternatively, a process was recently proposed by the same Applicant (see EP-A-2953280 according to Art. 54(3) EPC) which envisages initially spinning mixed yarns of extra-fine animal fibres (for example of cashmere) and silk fibres, doubling each of said mixed yarns with a respective yarn of water-soluble synthetic fibres, weaving the doubled yarns and finally dissolving or melting the water-soluble yarns to obtain a final textile of pure extra-fine animal fibres, in particular of pure extra-fine cashmere.

Once again, the doubling is carried out with opposite twist to that of the individual yarn, i.e. with an S twist.

In both cases, discontinuous water-soluble yarns are used, made up of fibres spun with cotton-type cut.

Aside from the undoubted and recognised value of the processes described above, there is the problem that the twisting performed in doubling the discontinuous water-soluble yarns in the opposite direction to that of the yarns of extra-fine fibres, besides requiring the use of relatively thick water-soluble yarns, substantially of the same fineness as the extra-fine yarns, gives rise to an effect known as "piling", which the male clients having beards and hair which can cause deterioration of the textile by rubbing, consider annoying.

JP-A- 55 098936 discloses a method for manufacturing a worsted crepe fabric.

US-A-2 592 153 discloses a process for manufacturing a textile fabric in which a wool yarn is twisted together with a synthetic filament having a fineness much lower than that of the wool fabric. The composite yarns are woven or knitted and the synthetic filament is then dissolved in an alkaline bath.

GB-A-1 068 662 discloses a method for making a bulky yarn starting by combining a bulky stretchable yarn of a substantially solid structure with a substantially unstretchable yarn and with a binding yarn. At least one of the unstretchable yarn and the binding yarn are made of a synthetic material which may be dissolved in an aqueous acid solution.

EP-A-1 245 706 discloses a process for manufacturing a worsted wool fabric in which a continuous filament of lower fineness is wrapped on a single wool yarn of higher fineness.

The object of the present invention has now been to create a process which enables the weaving of yarns in extra-fine animal fibres, particularly in cashmere fibres, using thinner water-soluble threads and reducing the "piling" effect to a minimum.

In view of this object, the process according to the present invention is characterised by comprising the succession of stages recited in claim 1.

By the use of continuous synthetic filaments subjected to slight doubling which matches that of the yarns with extra-fine animal fibres, it is possible industrially to obtain textiles in extra-fine animal fibres, particularly in cashmere fibres, losing slightly in softness by comparison with the known processes described above, but reducing to a minimum or actually eliminating the "piling" effect, to the great advantage of pleasantness of the finished product, and of greater durability.

The starting yarns can be of extra-fine animal fibres only, particularly of cashmere, or can be mixed yarns (in so-called "intimate mixture") of extra-fine animal fibres, for example of cashmere, and silk fibres. In both cases the yarns have a fineness of between 50 and 200 dtex.

Considering extra-fine animal fibres with a Z spinning twist of 1100 turns per linear metre, the twist for doubling the continuous filaments is a Z twist of about 200 turns per linear metre.

An embodiment of the process according to the present invention will now be described in detail with reference to the attached drawings, in which:
figure 1 shows a yarn with extra-fine animal fibres, in particular extra-fine cashmere fibres, doubled with a continuous synthetic filament, in particular of polyvinyl material, soluble in slightly acidic liquid solution at high temperature;
figure 2 shows a portion of a raw textile obtained by weaving yarns with extra-fine animal fibres doubled with continuous synthetic filaments as in figure 1;
figure 3 shows the same portion of textile after the dissolution of the synthetic filaments.

1 indicates a starting yarn with extra-fine animal fibres which are not industrially weavable. Yam 1 can be made up of extra-fine animal fibres only, particularly of cashmere, or can be a mixed yarn 1 of extra-fine animal fibres and silk fibres, for example of composition 80%WS (cashmere) - 20%SE (silk) with an extra-fine fineness of 66 dtex. Yam 1 is made using traditional spinning with a Z twist of 1100 turns per linear metre.

Yam 1 is doubled with a continuous synthetic filament 2, made in polyvinyl material (PVA), i.e. soluble in slightly acidic aqueous solution at high temperature. Continuous synthetic material 2 is of the same fineness as yarn 1, as illustrated in figures 1 and 2.

Doubling is performed with a twist in the same direction as that of yarns 1, i.e. with a Z twist. The doubling twist is of low level, of about 200 turns per linear metre, so as not to create strength problems for yarns 1, and so as to obtain good softness for the final product, accompanied by an almost total absence of "piling".

As shown in figure 2, an appropriate number of doubled combinations 3, each made up of a yarn 1 of pure extra-fine animal fibres or a mixture of extra-fine animal fibres and silk fibres and a continuous water-soluble synthetic filament 2, subsequently undergoes traditional warp and weft weaving (or on a circular machine of Jersey type), in which the synthetic filaments 2 function as a support to enable the weaving of yarns 1, otherwise not industrially weavable.

The raw textile thus created, which can be in any weave such as plain, twill or jacquard, clearly has the same composition as doubled combinations 3.

This raw textile then undergoes a stage of purging by a dyeing-type process, in which it is immersed in an aqueous solution of about 50 litres per kilogram of polyvinyl with a slightly acid pH (about 4.5) at a temperature of between 30°C and 100°C (depending on the nature of the PVA yarn).

The synthetic filaments 2 are thus eliminated by dissolution or melting, leaving a final textile (fig. 3) composed exclusively of yarns 1 and therefore having a final composition with a fineness of 66 dtex, which is impossible to achieve industrially with traditional techniques.

As a result of the slight Z twist imparted by the doubling in the same direction as the twist of yarns 1, after the dissolution of the synthetic yarns 2 the remaining yarn 1 has a twist which is the sum of the twists from spinning and doubling, in other words in the example under consideration a twist of 1300 Z, but it is sufficiently low as to make the final textile soft and at the same time to produce a considerable reduction in the "piling" effect.

## Claims

1. A process for the production of a textile in animal fibre yarns having a fineness between 50 and 200 dtex, comprising the following succession of stages:
a) spinning of yarns (1) containing animal fibres, the spun yarns (1) having a fineness between 50 and 200 dtex and a Z twist of 1100 turns per linear metre;
b) doubling of each spun yarn (1) with a respective continuous PVA (polyvinyl alcohol) synthetic filament (2) soluble in a liquid solution with about 4.5 pH at a temperature between 30°C and 100°C, said synthetic PVA filament (2) being substantially of the same fineness as the spun yarn (1), said doubling being executed with a Z twisting of about 200 turns per linear metre;
c) weaving of the doubled spun yarns (1) and filaments (2);
d) dissolution of said synthetic PVA filaments (2) by means of a liquid solution with about 4.5 pH at a temperature between 30°C and 100°C.

2. A process according to claim 1, **characterised in that** said spun yarns (1) are made of animal fibres only.

3. A process according to claim 1, **characterised in that** said spun yarns (1) are mixed yarns of animal fibres and silk fibres.

4. A process according to any of claims 1 to 3, **characterised in that** said animal fibres are cashmere fibres.

5. A process according to claim 3, **characterised in that** said mixed yarns (1) have a composition of 80% cashmere and 20% silk.

## Patentansprüche

1. Verfahren zur Herstellung eines Gewebes aus tierischen Fasergarnen, welche eine Feinheit zwischen 50 und 200 dtex haben, wobei das Verfahren die folgenden aufeinander folgenden Schritte aufweist:
a) Spinnen von Garnen (1), welche tierische Fasern enthalten, wobei die gesponnenen Garne (1) eine Feinheit zwischen 50 und 200 dtex und eine Z-Verdrillung von 1100 Windungen pro Meter Länge haben;
b) Verdoppeln des jeweiligen gesponnenen Garns (1) mit einem entsprechenden durchgehenden synthetischen Filament (2) aus PVA (Polyvenylalkohol), welches in einer flüssigen Lösung mit etwa 4,5 pH bei einer Temperatur zwischen 30°C und 100°C löslich ist, wobei das synthetischen PVA-Filament (2) im wesentlichen die gleiche Feinheit wie das gesponnene Garn (1) hat und das Verdoppeln mit einer Z-Verdrillung von etwa 200 Windungen pro Meter Länge ausgeführt wird;
c) Weben des doppelt gesponnenen Garns (1) und des Filaments (2);
d) Auflösen der synthetischen PVA-Filamente (2) mit Hilfe einer flüssigen Lösung mit etwa 4,5 pH bei einer Temperatur zwischen 30°C und 100°C.

2. Verfahren nach Anspruch 1, **dadurch gekennzeichnet, dass** die gesponnenen Garne (1) nur aus tierischen Fasern bestehen.

3. Verfahren nach Anspruch 1, **dadurch gekennzeichnet, dass** die gesponnenen Garne (1) Mischgarne aus tierischen Fasern und Seidenfasern sind.

4. Verfahren nach einem der Ansprüche 1 bis 3, **dadurch gekennzeichnet, dass** die tierischen Fasern Kashmirfasern sind.

5. Verfahren nach Anspruch 3, **dadurch gekennzeichnet, dass** die Mischgarne (1) eine Zusammensetzung von 80% Kashmir und 20% Seide haben.

## Revendications

1. Procédé pour la production d'un textile en fils de fibres animales ayant une finesse comprise entre 50 et 200 dtex, comprenant la succession suivante d'étapes consistant à :
a) filer des fils (1) contenant des fibres animales, les fils filés (1) ayant une finesse comprise entre 50 et 200 dtex et une torsion Z de 1100 tours par mètre linéaire ;
b) doubler chaque fil filé (1) avec un filament synthétique en PVA (alcool polyvinylique) continu (2) soluble dans une solution liquide avec un pH d'environ 4,5 à une température comprise entre 30°C et 100°C, ledit filament synthétique en PVA (2) étant sensiblement de la même finesse que le fil filé (1), ledit doublage étant réalisé avec une torsion Z d'environ 200 tours par mètre linéaire ;
c) tisser les fils filés (1) et les filaments (2) doublés ;
d) dissoudre lesdits filaments synthétiques en PVA (2) au moyen d'une solution liquide avec un pH d'environ 4,5 à une température comprise entre 30°C et 100°C.

2. Procédé selon la revendication 1, **caractérisé en ce que** lesdits fils filés (1) sont réalisés uniquement avec des fibres animales.

3. Procédé selon la revendication 1, **caractérisé en ce que** lesdits fils filés (1) sont des fils mélangés de fibres animales et des fibres de soie.

4. Procédé selon l'une quelconque des revendications 1 à 3, **caractérisé en ce que** lesdites fibres animales sont des fibres de cachemire.

5. Procédé selon la revendication 3, **caractérisé en ce que** lesdits fils mélangés (1) ont une composition de 80 % de cachemire et de 20 % de soie.
